



US005204212A

# United States Patent [19]

Tahon

[11] Patent Number: 5,204,212  
[45] Date of Patent: Apr. 20, 1993

[54] PROCESSING LIQUID FOR THE SILVER  
SALT DIFFUSION TRANSFER PROCESS  
CONTAINING  
3-(N,N-DIETHYLAMINO)PROPANE-1,2-  
DIOL

[75] Inventor: Jean-Pierre D. Tahon, Louvain,  
Belgium

[73] Assignee: Agfa-Gevaert, N.V., Mortsel,  
Belgium

[21] Appl. No.: 813,660

[22] Filed: Dec. 27, 1991

[30] Foreign Application Priority Data

Jan. 21, 1991 [EP] European Pat. Off. .... 91200111.2

[51] Int. Cl.<sup>5</sup> ..... G03C 5/54; G03C 5/30;  
G03C 5/38

[52] U.S. Cl. ..... 430/249; 430/244;  
430/251; 430/455; 430/456; 430/486; 430/487;  
430/490; 430/492

[58] Field of Search ..... 430/233, 244, 249, 251,  
430/455, 456, 486, 487, 489, 490, 492, 419, 429

[56]

## References Cited

### U.S. PATENT DOCUMENTS

|           |         |                       |         |
|-----------|---------|-----------------------|---------|
| 3,576,633 | 4/1971  | Henn et al. ....      | 430/489 |
| 3,619,185 | 11/1971 | Kasman ....           | 430/456 |
| 4,147,543 | 4/1979  | Kubotera et al. ....  | 430/244 |
| 4,568,634 | 2/1986  | Hayashi ....          | 430/249 |
| 4,632,896 | 12/1986 | Tsubai et al. ....    | 430/249 |
| 4,649,096 | 3/1987  | Tsubai et al. ....    | 430/249 |
| 4,668,605 | 5/1987  | Okutsu et al. ....    | 430/489 |
| 4,740,452 | 4/1988  | Okutsu et al. ....    | 430/486 |
| 5,063,136 | 11/1991 | De Keyzer et al. .... | 430/249 |

Primary Examiner—Richard L. Schilling  
Attorney, Agent, or Firm—Breiner & Breiner

[57]

## ABSTRACT

An aqueous alkaline processing liquid suitable for use in the silver complex diffusion transfer reversal (DTR-) process, wherein said liquid contains 3-(N,N-diethylamino)propane-1,2-diol and contains phosphate ions in a concentration of not more than 0.03 mol/l.

10 Claims, No Drawings

**PROCESSING LIQUID FOR THE SILVER SALT DIFFUSION TRANSFER PROCESS CONTAINING 3-(N,N-DIETHYLAMINO)PROPANE-1,2-DIOL**

**1. FIELD OF THE INVENTION**

The present invention relates to a processing liquid suitable for use in the silver complex diffusion transfer reversal process, hereinafter called DTR-process.

**2. BACKGROUND OF THE INVENTION**

The DTR-process initially intended for office copying purposes has found now wide application in the graphic art field, more particularly in the production of screened prints from continuous tone originals.

For the latter purpose it is particularly important that the processing characteristics remain steady for a large set of prints and that the gradation, optical density (transmission density in the case of film material and reflection density in the case of opaque material e.g. paper material) and the neutrality of the colour tone (black) of the screen dots in the screened prints satisfy graphic art standards which are particularly high compared with normal copying.

The principles of the silver complex diffusion transfer reversal process have been described e.g. in U.S. Pat. No. 2,352,014 and in the book "Photographic Silver Halide Diffusion Processes" by André Rott and Edith Weyde—The Focal Press—London and New York, (1972).

In the DTR-process non-developed silver halide of an image-wise exposed photographic silver halide emulsion layer material is transformed with a so-called silver solvent into soluble silver complex compounds which are allowed to diffuse into an image-receiving element and are reduced therein with a developing agent, generally in the presence of physical development nuclei, to form a silver image having reversed image density values with respect to the silver image obtained in the exposed photographic material.

The developing agent or a mixture of developing agents can be present in an alkaline processing solution and/or in the photographic silver halide emulsion layer material. In case the developing agent or a mixture of developing agents is contained in the photographic silver halide emulsion material, the processing solution can be merely an aqueous alkaline solution that initiates and activates the development.

Suitable developing agents for the exposed silver halide are e.g. hydroquinone-type and 1-phenyl-3-pyrazolidone-type developing agents as well as p-monomethylaminophenol.

The silver halide solvent, mostly sodium thiosulphate, may be supplied from the non-light-sensitive image-receiving element as mentioned above, but it is normally at least partly already present in the alkaline processing solution.

The alkaline processing solution usually contains sufficient alkaline substances to bring the pH above 10, e.g. sodium hydroxide, sodium carbonate and a great many other compounds which can raise the pH, for example borax, tertiary sodium phosphate, lithium hydroxide and amines, particularly alkanolamines.

The use of alkanolamines in processing solutions for DTR is disclosed in U.S. Pat. No. 4,568,634. However the there disclosed processing solutions contain phosphate salts in substantial amounts which is undesirable for ecological reasons. It is further known that phos-

phates may inhibit the swelling of gelatin, reduce the gradation and increase the stain in the image some time after the preparation of the processing solution.

Processing solutions for DTR substantially free of phosphate are disclosed in U.S. Pat. No. 4,632,896 and the European patent applications EP 397925, EP 397926, EP 397927 and EP 398435. However the processing characteristics of these processing solutions do not remain steady over a sufficient number of prints due to absorption of CO<sub>2</sub> from the air. Furthermore, although the processing characteristics of these fresh processing solutions are good it is still desirable to also improve these characteristics.

**3. SUMMARY OF THE INVENTION**

It is an object of the present invention to provide a processing liquid suitable for use in the silver complex diffusion transfer reversal process, which liquid has very low CO<sub>2</sub>-absorption resulting in more reproducible processing results over several day running of the processing liquid, shows a slow exhaustion, has excellent photographic properties and is substantially free of phosphate salts.

Another object of the present invention is to provide a method for carrying out the silver complex diffusion transfer reversal (DTR-) process wherein processing results are reproducible over several day running of said processing liquid especially with regard to development speed and image tone neutrality of the processed image-receiving element.

Other objects and advantages of this invention will become apparent from the description that follows.

According to the present invention a processing liquid suitable for use in the silver complex diffusion transfer reversal (DTR-) process is provided, wherein said liquid comprises 3-(N,N-diethylamino)propane-1,2-diol (hereinafter abbreviated as DEAPD) and a total amount of phosphate salts not larger than 0.03 mol/l.

According to the present invention a silver complex diffusion transfer reversal (DTR-) process is provided in which an image-wise exposed photographic silver halide emulsion layer is moistened with an aqueous alkaline processing liquid as defined above.

The moistening of said silver halide emulsion layer with said processing liquid proceeds while or before said layer is in relationship with an image-receiving layer to allow therein the transfer of complexed silver ions.

**4. DETAILED DESCRIPTION OF THE INVENTION**

Said tertiary alkanolamine DEAPD may be used in combination with a minor amount, i.e. not more than 0.2 mol, preferably less than 0.05 mol of an inorganic base per liter, e.g. not more than 2 g/l of sodium hydroxide to bring the pH of the processing liquid in the range of 10.5 to 13 without a substantial increase in CO<sub>2</sub>-absorption. For ecological reasons and to avoid a decrease in swelling of the hydrophilic colloid binder of the materials to be processed the present processing liquid is preferably completely free from phosphate ions.

DEAPD may also be used in combination with other alkanol amines being of the primary, secondary or tertiary type. Combinations with secondary and/or tertiary alkanol amines are preferred. Most preferably DEAPD is used as the single alkanol amine in a processing liquid for use in a silver diffusion transfer process.

The optimum pH of the processing liquid according to the present invention depends on the type of silver halide emulsion material to be developed, intended development time and processing temperature.

The processing temperature may vary within broad ranges but is preferably in the range of 10° to 35° C.

The silver halide developing agent used in the process and processing liquid according to the present invention is preferably a p-dihydroxybenzene compound, e.g. hydroquinone, methylhydroquinone or 10 chlorohydroquinone, preferably in combination with an auxiliary developing agent being a 1-phenyl-3-pyrazolidinone-type developing agent and/or p-monomethylaminophenol. When fairly low gradation images for continuous tone reproduction have to be 15 produced preference is given to developing agent combinations as described in U.S. Pat. Nos. 3,985,561 and 4,242,436.

According to the present invention the hydroquinone-type developing agents are present in the processing liquid in an amount of 0.05 to 0.25 mol per liter. 1-Phenyl-3-pyrazolidinone type developing agents may be present in an amount of  $1.8 \times 10^{-3}$  to  $2.0 \times 10^{-2}$  mol per liter. Particularly useful 1-phenyl-3-pyrazolidinone developing agents are 1-phenyl-3-pyrazolidinone, 1-phenyl-4-monomethyl-3-pyrazolidinone, 1-phenyl-4,4-dimethyl-3-pyrazolidinone, and 1-phenyl-4-methyl-4-hydroxymethyl-3-pyrazolidinone. The latter type of developing agents are advantageously present in the image receiving element.

A preferred quantitative combination of hydroquinone and at least one secondary or auxiliary developing agent of the class of 1-phenyl-3-pyrazolidinones and p-N-methyl-aminophenol comprises hydroquinone in an amount not lower than 0.078 mol per liter of aqueous alkaline solution and the secondary developing agent(s) in an amount not lower than 0.0080 mole per liter, the molar ratio of hydroquinone to said secondary developing agent(s) not being lower than 9.7. Most preferred amounts of hydroquinone are in the range of 0.15 mole to 0.20 mole per liter and most preferred amounts of secondary developing agent(s) in the range of 0.015 to 0.020 mole per liter.

According to a first embodiment said processing liquid contains said tertiary alkanolamine **DEAPD** and (a) developing agent(s) for silver halide development and none of such agents are present in the exposed photographic silver halide emulsion layer material and/or in the image-receiving element prior to said development.

According to a second embodiment at least part of the developing agent(s) is present in the photographic silver halide emulsion layer material and/or the image-receiving material before the material is photo-exposed and reaches the developable silver halide by diffusion with the aid of said processing liquid.

When incorporated in the photographic material, the developing agent(s) can be present in the silver halide emulsion layer or are preferably present in a hydrophilic colloid layer in water-permeable relationship therewith, e.g. in the antihalation layer adjacent to the silver halide emulsion layer of the photosensitive element.

A processing liquid that is initially free from developing agent(s) is called hereinafter "activator liquid".

As a preservative the present processing liquid contains sulphite ions which preferably originate from an alkali metal sulphite such as potassium or sodium sul-

phite, but may originate likewise from a sulphite precursor, e.g. aldehyde bisulphite such as formaldehyde bisulphite, or mixtures of such sulphites. The amount of sulphite ions is preferably between 16 and 76 g per liter.

For the DTR-process a silver halide solvent is indispensable. It may be supplied from the non-light-sensitive image-receiving element, but it is normally at least partly present already in the alkaline processing solution.

The silver halide solvent, which acts as a complexing agent for silver halide, preferably is a water-soluble thiosulphate or thiocyanate, e.g. sodium, potassium or ammonium thiosulphate or thiocyanate or mixtures thereof.

When present in the alkaline processing solution, the molar amount of thiosulphate compound is preferably in the range of 0.03 to 0.13 mol/l.

Other useful silver halide solvents are described in the book "The Theory of the Photographic Process" edited by T. H. James, 4th edition, p. 474-475 (1977), in particular sulphites and uracil. Further interesting silver halide solvents are described in U.S. Pat. Nos. 2,857,276 and 4,297,430, in particular cyclic imides such as 5,5-dialkylhydantoins. Still further are mentioned alkyl sulphones and amines and alkanolamines which also act as silver halide solvents. Mixtures of silver halide solvents may be used in order to control the speed of silver complexing and following speed of transfer of the silver complexes, especially in the case of so-called mono-sheet elements as referred to hereinafter.

The alkaline processing solution preferably also contains (a) silver image toning agent(s) providing a neutral (black) image tone to the DTR-produced silver image in the image-receiving material. A survey of suitable toning agents is given in the above mentioned book of André Rott and Edith Weyde, p. 61-65, preference being given to 1-phenyl-1H-tetrazole-5-thiol, also called 1-phenyl-5-mercapto-tetrazole, tautomeric structures and derivatives thereof such as

1-(2,3-dimethylphenyl)-5-mercaptop-tetrazole,  
 1-(3,4-dimethylcyclohexyl)-5-mercaptop-tetrazole,  
 1-(4-methylphenyl)-5-mercaptop-tetrazole,  
 1-(3-chloro-4-methylphenyl)-5-mercaptop-tetrazole,  
 1-(3,4-dichlorophenyl)-5-mercaptop-tetrazole.

Further particularly useful toning agents are of the class of thiohydantoins, preferably a compound corresponding to the following structural formula:



wherein: R<sup>11</sup> represents an allyl group, and each of R<sup>12</sup> and R<sup>13</sup> which may be the same or different represents an alkyl group, e.g. methyl group.

Other particularly useful silver image toning agents are in the class of phenyl substituted mercapto-triazoles, a preferred representative corresponding to the following structural formula:



Still further toning agents suitable for use in accordance with the present invention are the toning agents described in the European patent applications 218752, 208346, 218753 and U.S. Pat. No. 4,683,189.

For DTR-processing the aqueous alkaline processing solution according to the present invention may comprise (a) toning agent(s) in a concentration in a range e.g. from 30 mg to 200 mg per liter. Said toning agents may also at least partially be present in the image receiving layer and/or in a layer in water permeable relationship therewith.

Other additives for the processing solution are thickening agents, e.g. hydroxyethylcellulose and carboxymethylcellulose, fog inhibiting agents, e.g. potassium bromide, potassium iodide and a benzotriazole, calcium sequestering compounds, wetting agents, e.g. block copolymers of ethyleneoxide and propylene oxide, anti-sludge agents, and hardeners including latent hardeners.

The DTR-image can be formed in the image-receiving layer of a sheet or web material being a separate element with respect to the photographic silver halide emulsion material or in a so-called single-support-element, also called mono-sheet element or unitary DTR-material, which contains at least one photographic silver halide emulsion layer and the image-receiving layer in waterpermeable relationship therewith, e.g. on top of each other or separated by a thin waterpermeable striping layer or alkali-degradable interlayer as described e.g. in U.S. Pat. No. 3,684,508 or wherein the photographic silver halide emulsion layer is optically masked from the image-receiving layer, e.g. with a white waterpermeable pigment layer as described e.g. in U.S. Pat. Nos. 3,607,270 and 3,740,220.

The support of the image receiving material may be opaque or transparent, e.g. a paper support or resin support.

The image receiving layer comprises for best imaging results physical development nuclei normally in the presence of a protective hydrophilic colloid, e.g. gelatin and/or colloidal silica.

Preferred development nuclei are sulphides of heavy metals e.g. sulphides of antimony, bismuth, cadmium, cobalt, lead, nickel, palladium, platinum, silver, and zinc. Especially suitable development nuclei are NiS- $\text{Ag}_2\text{S}$  nuclei as described in U.S. Pat. No. 4,563,410. Other suitable development nuclei are salts such as e.g. selenides, polyselenides, polysulphides, mercaptans, and tin (II) halides. Heavy metals or salts thereof and fogged silver halide are suitable as well. The complex salts of lead and zinc sulphides are active both alone and when mixed with thioacetamide, dithiobiuret, and dithiooxamide. Heavy metals, preferably silver, gold, platinum, palladium, and mercury can be used in colloidal form.

The image-receiving element may contain in operative contact with the development nuclei thioether compounds, e.g. those described in DE-P 1,124,354, in U.S. Pat. Nos. 4,013,471 and 4,072,526, and in published European Patent Application (EP-A) 0 026 520.

Most of the DTR-positive materials now available on the market are composed of two or even three layers.

Such materials normally contain on top of the nuclei containing layer a layer which itself contains no nuclei and otherwise has the same composition as the nuclei containing layer and mainly serves to ensure good contact between the negative and positive material during transfer. Moreover, after drying this layer provides a protective coating for the image receiving layer containing the silver image. It further prevents bronzing or pluming of the black image areas in preventing the protruding of silver from the image receiving layer in the form of a glossy silver mirror (ref. the above mentioned book p. 50).

According to a preferred embodiment the processing liquid and/or the image-receiving element contains at least one image toning agent e.g. of the type referred to hereinbefore. In said case the image toning agent(s) may gradually transfer by diffusion from said image-receiving element into the processing liquid and keep therein the concentration of said agents almost steady. In practice such can be realized by using the above defined silver image toning agents in a coverage in the range from 1 mg/m<sup>2</sup> to 20 mg/m<sup>2</sup> in a hydrophilic waterpermeable colloid layer.

According to a practical embodiment in the image-receiving element the development nuclei containing layer and/or hydrophilic colloid layer in waterpermeable relationship or a back layer at the side of the support opposite to that carrying the image receiving layer contains at least part of the silver image toning agents. Such procedure results actually in automatic replenishment of toning agent in the processing liquid. The same applies at least partly for the replenishment of the developing agent(s) and silver halide complexing agent(s).

According to another embodiment at least a part of said silver image toning agents is present in the silver halide emulsion material to be developed. Such means that in a practical embodiment at least one of the image toning agents may be used in a hydrophilic waterpermeable colloid layer, e.g. antihalation layer at the side of the support opposite to the side coated with a silver halide emulsion layer or between the support and the silver halide emulsion layer. The coverage of said silver image toning agents in said antihalation layer is preferably in the range of 1 mg/m<sup>2</sup> to 20 mg/m<sup>2</sup>.

The transfer behaviour of the complexed silver largely depends on the thickness of the image-receiving layer and the kind of binding agent or mixture of binding agents used in the nuclei containing layer. In order to obtain a sharp image with high spectral density the reduction of the silver salts diffusing into the image receiving layer must take place rapidly before lateral diffusion becomes substantial.

An image-receiving material satisfying said purpose is described in U.S. Pat. No. 4,859,566 and is particularly suitable for being processed with an aqueous alkaline processing liquid according to the present invention.

An image-receiving material of this type is very suitable for use with a processing liquid according to the present invention and contains a water-impermeable support coated with (1) an image-receiving layer containing physical development nuclei dispersed in a waterpermeable binder and (2) a waterpermeable top layer free from development nuclei and containing a hydrophilic colloid, in such a way that:

- (i) the total solids coverage of said two layers (1) and (2) is at most 2 g/m<sup>2</sup>,

- (ii) in layer (1) the coverage of the nuclei is in the range of 0.1 mg/m<sup>2</sup> to 10 mg/m<sup>2</sup>, and the coverage of binder is in the range of 0.4 to 1.5 g/m<sup>2</sup>, and
- (iii) in said top layer (2) the coverage of hydrophilic colloid is in the range of 0.1 to 0.9 g/m<sup>2</sup>.

The coating of said layers proceeds preferably with slide hopper coater or curtain coater known to those skilled in the art.

A white appearance of the image background even when a yellow stain should appear on storage is obtained by incorporation of optical brightening agents in the support, image-receiving layer and/or interlayer between the support and the image-receiving layer.

According to a particular embodiment the nuclei containing layer (1) is present on a nuclei-free underlying hydrophilic colloid undercoat layer or undercoat layer system having a coverage in the range of 0.1 to 1 g/m<sup>2</sup> of hydrophilic colloid, the total solids coverage of layers (1) and (2) together with the undercoat being at most 2 g/m<sup>2</sup>.

The undercoat optionally incorporates substances that improve the image quality, e.g. incorporates a substance improving the image-tone or the whiteness of the image background. For example, the undercoat may contain a fluorescent substance, silver complexing agent(s) and/or development inhibitor releasing compounds known for improving image sharpness.

According to a special embodiment the image-receiving layer (1) is applied on an undercoat playing the role of a timing layer in association with an acidic layer serving for the neutralization of alkali of the image-receiving layer. By the timing layer the time before neutralization occurs is established, at least in part, by the time it takes for the alkaline processing composition to penetrate through the timing layer. Materials suitable for neutralizing layers and timing layers are disclosed in Research Disclosure July 1974, item 12331 and July 1975, item 13525.

In the image-receiving layer (1) and/or in said top layer (2) and/or in an undercoat gelatin is used preferably as hydrophilic colloid. In layer (1) gelatin is present preferably for at least 60% by weight and is optionally used in conjunction with an other hydrophilic colloid, e.g. polyvinyl alcohol, cellulose derivatives, preferably carboxymethyl cellulose, dextran, galactomannans, 45 alginic acid derivatives, e.g. alginic acid sodium salt and/or watersoluble polyacrylamides. Said other hydrophilic colloid may be used also in the top layer for at most 10% by weight and in the undercoat in an amount lower than the gelatin content.

The image-receiving layer and/or a hydrophilic colloid layer in water-permeable relationship therewith may comprise a silver halide developing agent and/or silver halide solvent, e.g. sodium thiosulphate in an amount of approximately 0.1 g to approximately 4 g per 55 m<sup>2</sup>.

The image-receiving layer or a hydrophilic colloid layer in water-permeable relationship therewith may comprise colloidal silica.

The image-receiving layer may contain as physical development accelerators, in operative contact with the developing nuclei, thioether compounds such as those described e.g. in DE-A-1,124,354; U.S. Pat. Nos. 4,013,471; 4,072,526; and in EP 26520.

When applying an optical brightening agent in the image-receiving material preference is given to an optical brightening agent that is inherently by its structure resistant to diffusion or is made resistant to diffusion by

use in conjunction with another substance wherein it is dissolved or whereto it is adsorbed.

For example, to make an optical brightening agent resistant to diffusion one of the following techniques 5 may be applied.

According to a first technique known from colour photography the optical brightening compound is substituted with a long chain aliphatic residue and ionomeric residue as is known in the synthesis of diffusion resistant colour couplers.

According to a second technique an optical brightening agent of the oleophilic type is incorporated in droplets of a water-immiscible solvent, so-called "oil-former", e.g. dibutylphthalate.

According to a third technique the optical brightening agent is used in conjunction with a polymeric hydrophilic colloid adsorber, a so-called trapping agent, e.g. poly-N-vinylpyrrolidinone as described e.g. in U.S. Pat. Nos. 3,650,752, 3,666,470 and 3,860,427 and published European patent application 0 106 690.

According to a fourth technique latex compositions are used wherein latex particles are loaded, i.e. contain in dissolved and/or adsorbed state an optical brightening agent as described e.g. in German Offenlegungsschrift (DE-OS) 1,597,467 and in U.S. Pat. No. 4,388,403.

The image-receiving layer and/or other hydrophilic colloid layer of an image-receiving material used in a DTR-process according to the present invention may 30 have been hardened to some extent to achieve enhanced mechanical strength. Appropriate hardening agents for hardening the natural and/or synthetic hydrophilic colloid binding agents in the image-receiving layer include e.g. formaldehyde, glyoxal, mucochloric acid, 35 and chrome alum. Other suitable hardening agents for hardening the hydrophilic colloid binding agents in the image-receiving layer are vinylsulphonyl hardeners, e.g. as described in Research Disclosure 22,507 of Jan. 1983.

According to a preferred embodiment hardening is effected by incorporating a hardener precursor in the image-receiving layer, the hardening of the hydrophilic colloid therein being triggered by the treatment with the alkaline processing liquid.

In the process of the present invention the image-receiving material can be used in the form of roll film or sheet film or in the form of a film pack e.g., for in-camera-processing.

The image-receiving material can be used in conjunction 50 with any type of photographic silver halide emulsion material suited for use in diffusion transfer reversal processing. The silver halide emulsion material may contain one or more hydrophilic colloid-silver halide emulsion layers.

In the photographic material to be processed after exposure with a processing solution according to the present invention whether or not in combination with a DTR-image-receiving material, the hydrophilic colloid silver halide emulsion layer can be coated from any 60 photosensitive silver halide emulsion comprising a hydrophilic colloid binder, which usually is gelatin. But instead of or together with gelatin, use can be made of one or more other natural and/or synthetic hydrophilic colloids, e.g. albumin, casein, zein, polyvinyl alcohol, alginic acids or salts thereof, cellulose derivatives such as carboxymethyl cellulose, modified gelatin, e.g. phthaloyl gelatin etc. The weight ratio of hydrophilic colloid binder to silver halide expressed as equivalent

amount of silver nitrate to binder is e.g. in the range of 1:1 to 10:1.

The photosensitive silver halide used in the present invention may comprise silver chloride, silver bromide, silver bromoiodide, silver chlorobromoiodide and the like, or mixtures thereof. To obtain a sufficiently high rate of solution of the silver halide and a satisfactory gradation necessary for graphic purposes a silver halide emulsion mainly comprising silver chloride is used preferably. This silver chloride emulsion may comprise minor amounts of silver bromide and/or silver iodide.

The silver halide emulsions may be coarse or fine grain and can be prepared by any of the well known procedures e.g. single jet emulsions, double jet emulsions such as Lippmann emulsions, ammoniacal emulsions, thiocyanate- or thioether-ripened emulsions such as those described in U.S. Pat. Nos. 2,222,264, 3,320,069, and 3,271,157. Surface image emulsions may be used or internal image emulsions may be used such as those described in U.S. Pat. Nos. 2,592,250, 3,206,313, and 3,447,927. If desired, mixtures of surface and internal image emulsions may be used as described in U.S. Pat. No. 2,996,382.

The silver halide particles of the photographic emulsions may have a regular crystalline form such as cubic or octahedral form or they may have a transition form. Regular-grain emulsions are described e.g. in J. Photogr. Sci., Vol. 12, No. 5, September/October 1964, pp. 242-251. The silver halide grains may also have an almost spherical form or they may have a tabular form (so-called T-grains), or may have composite crystal forms comprising a mixture of regular and irregular crystalline forms. The silver halide grains may have a multilayered structure having a core and shell of different halide composition. Besides having a differently composed core and shell the silver halide grains may comprise also different halide compositions and metal dopants inbetween.

Two or more types of silver halide emulsions that have been prepared differently can be mixed for forming a photographic emulsion for use in a photographic material treated with a processing liquid according to the present invention.

The average size of the silver halide grains may range from 0.2 to 1.2  $\mu$ m, and the size distribution can be homodisperse or heterodisperse. A homodisperse size distribution is obtained when 95% of the grains have a size that does not deviate more than 30% from the average grain size.

Apart from negative-working silver halide emulsions that are preferred for their high light-sensitivity, use can be made also of direct-positive silver halide emulsions that produce a positive silver image.

For instance, direct-positive emulsions of the type described in U.S. Pat. No. 3,062,651 may be employed. In direct-positive emulsions a non-hardening fogging agent such as stannous chloride and formamidine sulphonic acid can be used.

The emulsions can be chemically sensitized e.g. by adding sulphur-containing compounds during the chemical ripening stage e.g. allyl isothiocyanate, allyl thiourea, and sodium thiosulphate. Also reducing agents e.g. the tin compounds described in BE-A 493,464 and 568,687, and polyamines such as diethylene triamine or derivatives of aminomethane-sulphonic acid can be used as chemical sensitizers. Other suitable chemical sensitizers are noble metals and noble metal compounds such as gold, platinum, palladium, iridium,

ruthenium and rhodium. This method of chemical sensitization has been described in the article of R. KOSLOWSKY, Z. Wiss. Photogr. Photophys. Photochem. 46, 65-72 (1951).

5 The emulsions can also be sensitized with polyalkylene oxide derivatives, e.g. with polyethylene oxide having a molecular weight of 1000 to 20,000, or with condensation products of alkylene oxides and aliphatic alcohols, glycols, cyclic dehydration products of hexitols, alkyl-substituted phenols, aliphatic carboxylic acids, aliphatic amines, aliphatic diamines and amides. The condensation products have a molecular weight of at least 700, preferably of more than 1000. It is also possible to combine these sensitizers with each other as 10 described in BE-A 537,278 and GB-A 727,982.

The spectral photosensitivity of the silver halide can be adjusted by proper spectral sensitization by means of the usual mono- or polymethylene dyes such as acidic or basic cyanines, hemicyanines, oxonols, hemioxonols, 15 styryl dyes or others, also tri- or polynuclear methine dyes e.g. rhodacyanines or neocyanines. Such spectral sensitizers have been described by e.g. F. M. HAMER in "The Cyanine Dyes and Related Compounds" (1964) Interscience Publishers, John Wiley & Sons, New York.

The silver halide emulsions may contain the usual stabilizers e.g. homopolar or salt-like compounds of mercury with aromatic or heterocyclic rings such as mercaptotriazoles, simple mercury salts, sulphonium mercury double salts and other mercury compounds. 20 Other suitable stabilizers are azaindenes, preferably tetra- or penta-azaindenes, especially those substituted with hydroxy or amino groups. Compounds of this kind have been described by BIRR in Z. Wiss. Photogr. Photophys. Photochem. 47, 2-27 (1952). Other suitable 25 stabilizers are i.a. heterocyclic mercapto compounds e.g. phenylmercaptotetrazole, quaternary benzothiazole derivatives, and benzotriazole.

The silver halide emulsions may further contain either or not in combination with one or more developing 30 agents pH controlling ingredients, and other ingredients such as antifogging agents, development accelerators, wetting agents, and hardening agents for gelatin.

The silver halide emulsion layer may comprise light-screening dyes that absorb scattering light and thus 35 promote the image sharpness and, as a consequence thereof, the sharpness of the final printed copy. Light-absorbing dyes that can be used as light-screening dyes have been described in i.a. U.S. Pat. Nos. 4,092,168, 4,311,787, DE-A 2,453,217, and GB-A 7,907,440. More 40 details about the composition, preparation and coating of silver halide emulsions can be found in e.g. Product Licensing Index, Vol. 92, December 1971, publication 9232, p. 107-109.

As an interesting variant in the DTR-process the 45 silver halide emulsion may consist of a first light-sensitive silver halide emulsion in which a normal latent image is formed upon image-wise exposure and a second silver halide emulsion whose speed is so low that no or almost no latent image is formed therein. When the 50 low-speed silver halide emulsion and the light-sensitive silver halide emulsion are coated to form different layers, the resulting emulsion layers are arranged in DTR-processing in such a way that the low-speed emulsion is remotest from the image-receiving layer. It is also possible to coat one single layer comprising a mixture of both 55 types of emulsion.

Thanks to the combination of light-sensitive and low-speed emulsions a silver image having an enhanced

contrast can be obtained. Such may be explained by the fact that upon application of an aqueous alkaline solution to the image-wise exposed light-sensitive silver halide emulsion layer system in the presence of a developing agent and a silver halide solvent a silver image is formed in the image-receiving layer from the additionally obtained silver complexes in the low-speed emulsion layer. No image-background staining in the DTR-print takes place because the reduced silver of the light-sensitive emulsion forms a barrier for silver halide or complexes of the low-speed emulsion that would also tend to migrate towards the image-receiving element. As a result, the silver halide or complexes thereof diffusing from both the light-sensitive emulsion and the low-speed emulsion together build up said strengthened 15 high-contrast silver image in the image receiving layer.

As the sensitivity of the low speed emulsion must be low enough to be inert in the photo-exposure, no second ripening or after-ripening thereof is applied.

The low-speed emulsion may be a pure silver chloride emulsion or an emulsion of mixed silver halides comprising silver chloride e.g. a silver chlorobromide or chlorobromoiodide emulsion. However, the low-speed emulsion is preferably a silver chloride emulsion for the greater part. Preferably a fine-grain silver chloride having a particle size in the range of 50 to 500 nm is used.

In case a mixture of low-speed emulsion and of imaging emulsion is coated to form one single layer, the amount of low-speed emulsion may vary within wide limits. Favourable results can be obtained when the ratio of low-speed silver chloride-containing emulsion to image-forming emulsion, expressed in parts by weight of silver nitrate, ranges from 10:1 to 1:1. The amount of low-speed emulsion to be added depends i.a. 30 on its own nature, on the type of image-forming emulsion used, and on the effect desired. It can be determined easily by routineers in the art by making a few comparative tests.

The silver halide emulsion coated side of the photographic material can be provided with a top layer that contains hydrophilic colloids that form a waterpermeable layer. Such top layer is usually free of gelatin. Its nature is such that it does not inhibit or restrain the diffusion transfer of the complexed silver but acts e.g. as 45 an anti-stress layer. Appropriate hydrophilic binding agents for such top layer are e.g. methyl cellulose, the sodium salt of carboxymethyl cellulose, hydroxyethyl cellulose, hydroxyethyl starch, hydroxypropyl starch, sodium alginate, gum tragacanth, starch, polyvinyl alcohol, polyacrylic acid, polyacrylamide, poly-N-vinyl pyrrolidinone, polyoxyethylene, and copoly(methylvinylether/maleic acid). The thickness of this layer depends on the nature of the colloid used and the required mechanical strength. Such layer if present may 50 be transferred at least partially to the image-receiving layer without deleterious action on the image formation.

The development and diffusion transfer can be initiated in different ways e.g. by rubbing with a roller that has been wetted with the processing liquid, e.g. acts as meniscus coater, by wiping with an absorbent means e.g. with a plug of cotton or sponge, or by dipping the material to be treated in the liquid composition. Preferably, they proceed in an automatically operated apparatus such as the COPYPROOF (registered trade name of AGFA-GEVAERT N.V. Belgium) type CP 38, CP 380, CP 42 or CP 530 processors. The DTR-process is 55

normally carried out at a temperature in the range of 10° C. to 35° C.

The following examples illustrate the present invention without however, limiting it thereby. All parts, percentages and ratios are by weight unless otherwise indicated.

#### EXAMPLE 1

##### Preparation of Negative Working Silver Halide Emulsion Material (N)

A paper support having a weight of 110/m<sup>2</sup> being coated at both sides with a polyethylene layer was coated at one side with an antihalation layer on the basis of carbon black dispersed in gelatin wherein also hydroquinone and 1-phenyl-4-methyl-pyrazolidin-3-on were present in a coverage of 0.57 g/m<sup>2</sup> and 0.32 g/m<sup>2</sup>. On said antihalation layer an orthochromatically sensitized negative working gelatino silver halide emulsion layer containing an amount of silver chlorobromide (1.8 mol % bromide) equivalent to 2.0 g/m<sup>2</sup> of silver nitrate was coated. The average grain size of the silver chlorobromide was 0.3 microns. The silver halide emulsion layer was overcoated with a thin protective gelatin layer.

##### Preparation of Direct-Positive Working Silver Halide Emulsion Material (M)

The direct-positive working silver halide emulsion material (M) was prepared analogously to Material C of the Example of U.S. Pat. No. 4,144,064.

##### Preparation of Image-Receiving Material (A1)

One side of a paper support having a weight of 110 g/m<sup>2</sup> and being coated at both sides with a polyethylene layer was coated at a dry coverage of 2 g/m<sup>2</sup> with an image-receiving layer containing silver-nickel sulphide nuclei and gelatin. This layer was applied by slide hopper coating so that the nuclei were in an undermost coating of 1.3 g gelatin per m<sup>2</sup> and a top layer was provided of 0.7 g of gelatin per m<sup>2</sup>.

##### Preparation of Image-Receiving Material (A2)

To one side of a paper support having a weight of 110 g/m<sup>2</sup> and being coated at both sides with a polyethylene layer were coated at a dry coverage of 1.3 g/m<sup>2</sup> an image-receiving layer containing silver-nickel sulphide nuclei, an optical brightening agent, 75% of gelatin, 10% of carboxymethyl cellulose and 15% of a low molecular weight polyvinylalcohol and at a dry coverage of 0.7 g/m<sup>2</sup> a layer of gelatin.

##### Preparation of Image-Receiving Material (A3)

A subbed polyethylene terephthalate film support was coated at both sides at a dry coverage of 1.8 g/m<sup>2</sup> with an image-receiving layer containing silver-nickel sulphide nuclei dispersed in gelatin. This layer was applied by slide hopper coating so that the nuclei were in an undermost coating of 1.4 g gelatin per sq. m. is a top layer was provided of 0.4 g gelatin per m<sup>2</sup>.

#### Exposure Procedure

The photographic materials were exposed through a sensitometric wedge in a contact exposure apparatus operating with a light source having a colour temperature of 3200° K.

## DTR-Transfer Procedure

The exposed photographic materials were pre-moistened with the hereinafter defined processing liquids, the contact time with said liquid being 6 seconds before being pressed together with an image-receiving material as defined above. The transfer processor employed was a COPYPROOF (registered trade name of AGFA-GEVAERT N.V.) type CP 380. The transfer contact time was 30 seconds for the paper type image receiving materials and 60 seconds for the resin film type image receiving materials. Several transfers were carried out

gradient of the straight line portion of the sensitometric curve). The reflection density measurement proceeded according to American National Standard for Photography (Sensitometry) ANSI PH2.17-1985.

5 For the DTR-prints obtained on transparent resin film base image-receiving materials maximum transmission density was measured ( $D_{max}$  T), and the gamma value (maximum gradient of the straight line portion of the sensitometric curve). The transmission density measurement proceeded according to American National Standard for Photography (Sensitometry) ANSI PH2.19-1986.

| Ingredient  | Composition of processing solutions |       |       |                     |      |      |       |       |
|-------------|-------------------------------------|-------|-------|---------------------|------|------|-------|-------|
|             | Comparative solutions               |       |       | Inventive solutions |      |      |       |       |
|             | A                                   | B     | C     | D                   | E    | F    | G     | H     |
| I (g)       | 1.0                                 | 1.5   | 1.5   | 1.0                 | id   | id   | 1.5   | 1.5   |
| II (g)      | 2.0                                 | id    | id    | 2.0                 | id   | id   | id    | id    |
| III (g)     | 45.0                                | id    | 60.0  | 45.0                | id   | id   | id    | id    |
| IV (g)      | 14.0                                | id    | 12.0  | 14.0                | id   | 16.0 | 12.0  | id    |
| V (g)       | 0.5                                 | id    | 0.8   | 0.5                 | id   | id   | id    | id    |
| VI (g)      | 0.0                                 | 13.0  | 13.0  | 0.0                 | id   | id   | 13.0  | 13.0  |
| VII (g)     | 0.0                                 | 4.7   | 4.7   | 0.0                 | id   | id   | 4.7   | 4.7   |
| VIII (g)    | 0.1                                 | 0.080 | 0.07  | 0.1                 | id   | id   | 0.08  | 0.08  |
| IX (g)      | 0.02                                | 0.035 | 0.045 | 0.02                | id   | id   | 0.035 | 0.035 |
| MMEA (ml)   | 45.0                                | 20.0  | 30.0  | 32.1                | 16.1 | 0.0  | 24.1  | 0.0   |
| MDEA (ml)   | 30.0                                | 45.0  | 0.0   | 0.0                 | 0.0  | 0.0  | 0.0   | 0.0   |
| DEAPD (ml)  | 0.0                                 | 0.0   | 0.0   | 14.7                | 44.1 | 73.5 | 14.7  | 44.1  |
| NaOH (g)    | 0.0                                 | 2.0   | 2.0   | 0.0                 | 2.0  | 0.0  | 2.0   | 2.0   |
| Water up to | 11                                  | id    | id    | id                  | id   | id   | id    | id    |

I: Hydroxyethylcellulose

II: Ethylenediaminetetraacetic acid tetrasodium salt

III:  $Na_2SO_3$  (anhydrous)

IV:  $Na_2S_2O_3$  (anhydrous)

V: KBr

VI: Hydroquinone

VII: 1-Phenyl-4-methyl-3-pyrazolidinone

VIII: 1-Phenyl-5-mercapto-tetrazole

IX: 1-(3,4-Dichlorophenyl)-1H-tetrazole-5-thiol

MMEA is N-methyl-ethanolamine.

MDEA is N-methyl-diethanolamine.

at different processing liquid temperatures being 16°, 22° and 32° C. respectively.

The influence of the actual  $CO_2$ -absorption on the image quality was evaluated by processing sets of photographic materials (N) and (M) with image-receiving materials A1, A2 and A3, respectively with processing liquids that had been exposed before use to an atmosphere of 85% relative humidity containing 5000 ppm of  $CO_2$ . The  $CO_2$  atmosphere was obtained in a closed box with a  $CO_2$ -flow of 2.5 l/min under atmospheric pressure.

50 The obtained test wedge prints in the image-receiving materials were evaluated with regard to maximum density ( $D_{max}$ ) and gradation (gamma-value), the results of which are listed in the following Tables.

For the evaluation of the exhaustion of the processing liquid the following procedure was used. During 5 days each day 20 photographic materials (N) and (M) with image-receiving materials A1, A2 and A3 were processed. These results are also presented in the following tables.

## Evaluation

60 All wedge prints were measured on a densitometer MACBETH (registered trade name) type IR 924 behind visual filter, having following wavelength (nm)/optical density (D) characteristics: 700 nm/D=0; 600 nm/D=0.2; 500 nm/D=1.25; 420 nm/D=3.0.

65 For the DTR-prints obtained on paper base image-receiving materials maximum reflection density was measured ( $D_{max}R$ ), and the gamma value (maximum

TABLE 1

| Processing solution | Processing of photosensitive material N with image receiving materials A1, A2 and A3. Processing temperature: 16° C.; $CO_2$ -exposure: 0h; Number of materials that have been processed before: 0. |       |           |       |           |       |
|---------------------|-----------------------------------------------------------------------------------------------------------------------------------------------------------------------------------------------------|-------|-----------|-------|-----------|-------|
|                     | Mat. A1                                                                                                                                                                                             |       | Mat. A2   |       | Mat. A3   |       |
|                     | $D_{max}$                                                                                                                                                                                           | Gamma | $D_{max}$ | Gamma | $D_{max}$ | Gamma |
| A                   | 1.77                                                                                                                                                                                                | 27.0  | 1.72      | 24.2  | 4.26      | 18.0  |
| B                   | 1.86                                                                                                                                                                                                | —     | 1.84      | 21.0  | 3.92      | 17.0  |
| C                   | —                                                                                                                                                                                                   | —     | 1.86      | 23.0  | 3.96      | 17.0  |
| D                   | 1.86                                                                                                                                                                                                | 30.0  | 1.85      | 24.5  | 4.20      | 20.0  |
| E                   | 1.94                                                                                                                                                                                                | 29.0  | 1.96      | 26.0  | 4.09      | 21.0  |
| F                   | —                                                                                                                                                                                                   | —     | 2.00      | 24.3  | 4.11      | 18.0  |
| G                   | —                                                                                                                                                                                                   | —     | 1.89      | 22.0  | 4.11      | 17.0  |
| H                   | —                                                                                                                                                                                                   | —     | 1.96      | 19.0  | 3.75      | 18.0  |

TABLE 2

| Processing solution | Processing of photosensitive material N with image receiving materials A1, A2 and A3. Processing temperature: 22° C.; $CO_2$ -exposure: 0h; Number of materials that have been processed before: 0. |       |           |       |           |       |
|---------------------|-----------------------------------------------------------------------------------------------------------------------------------------------------------------------------------------------------|-------|-----------|-------|-----------|-------|
|                     | Mat. A1                                                                                                                                                                                             |       | Mat. A2   |       | Mat. A3   |       |
|                     | $D_{max}$                                                                                                                                                                                           | Gamma | $D_{max}$ | Gamma | $D_{max}$ | Gamma |
| A                   | 1.72                                                                                                                                                                                                | 33.0  | 1.66      | 31.4  | 3.94      | 18.0  |
| B                   | 1.76                                                                                                                                                                                                | —     | 1.80      | 24.0  | 4.07      | 16.0  |
| C                   | —                                                                                                                                                                                                   | —     | 1.79      | 31.0  | 4.09      | 17.0  |
| D                   | 1.79                                                                                                                                                                                                | 29.0  | 1.73      | 29.9  | 4.37      | 22.0  |
| E                   | 1.88                                                                                                                                                                                                | 27.0  | 1.85      | 31.3  | 4.28      | 21.0  |
| F                   | —                                                                                                                                                                                                   | —     | 1.88      | 23.5  | 4.10      | 19.0  |
| G                   | —                                                                                                                                                                                                   | —     | 1.82      | 28.0  | 4.14      | 17.0  |
| H                   | —                                                                                                                                                                                                   | —     | 1.96      | 21.0  | 3.90      | 18.0  |

TABLE 3

| Processing of photosensitive material N with image receiving materials A1, A2 and A3. Processing temperature: 32° C.; CO <sub>2</sub> -exposure: 0h; Number of materials that have been processed before: 0. |                  |       |                  |       |                  |       |   |
|--------------------------------------------------------------------------------------------------------------------------------------------------------------------------------------------------------------|------------------|-------|------------------|-------|------------------|-------|---|
| Processing solution                                                                                                                                                                                          | Mat. A1          |       | Mat. A2          |       | Mat. A3          |       |   |
|                                                                                                                                                                                                              | D <sub>max</sub> | Gamma | D <sub>max</sub> | Gamma | D <sub>max</sub> | Gamma |   |
| A                                                                                                                                                                                                            | 1.66             | 36.0  | 1.61             | 36.5  | 3.67             | 19.0  | 5 |
| B                                                                                                                                                                                                            | 1.73             | —     | 1.73             | 34.0  | 4.07             | 17.0  |   |
| C                                                                                                                                                                                                            | —                | —     | 1.65             | 37.0  | 4.09             | 16.0  |   |
| D                                                                                                                                                                                                            | 1.70             | 36.0  | 1.68             | 35.2  | 4.36             | 21.0  |   |
| E                                                                                                                                                                                                            | 1.77             | 33.0  | 1.75             | 34.6  | 4.40             | 21.0  |   |
| F                                                                                                                                                                                                            | —                | —     | 1.81             | 28.1  | 3.82             | 21.0  |   |
| G                                                                                                                                                                                                            | —                | —     | 1.73             | 33.0  | 4.12             | 16.0  |   |
| H                                                                                                                                                                                                            | —                | —     | 1.88             | 31.0  | 4.05             | 17.0  |   |

TABLE 4

| Processing of photosensitive material M with image receiving materials A2 and A3. Processing temperature: 16° C.; CO <sub>2</sub> -exposure: 0h; Number of materials that have been processed before: 0. |                  |       |                  |       |  |  |  |
|----------------------------------------------------------------------------------------------------------------------------------------------------------------------------------------------------------|------------------|-------|------------------|-------|--|--|--|
| Processing solution                                                                                                                                                                                      | Mat. A2          |       | Mat. A3          |       |  |  |  |
|                                                                                                                                                                                                          | D <sub>max</sub> | Gamma | D <sub>max</sub> | Gamma |  |  |  |
| B                                                                                                                                                                                                        | 1.73             | 9.7   | 3.51             | 10.5  |  |  |  |
| C                                                                                                                                                                                                        | 1.83             | 10.6  | 3.09             | 12.4  |  |  |  |
| G                                                                                                                                                                                                        | 1.86             | 13.1  | 3.83             | 11.4  |  |  |  |
| H                                                                                                                                                                                                        | 1.93             | 8.4   | 3.23             | 9.8   |  |  |  |

TABLE 5

| Processing of photosensitive material M with image receiving materials A1, A2 and A3. Processing temperature: 22° C.; CO <sub>2</sub> -exposure: 0h; Number of materials that have been processed before: 0. |                  |       |                  |       |  |  |    |
|--------------------------------------------------------------------------------------------------------------------------------------------------------------------------------------------------------------|------------------|-------|------------------|-------|--|--|----|
| Processing solution                                                                                                                                                                                          | Mat. A2          |       | Mat. A3          |       |  |  |    |
|                                                                                                                                                                                                              | D <sub>max</sub> | Gamma | D <sub>max</sub> | Gamma |  |  |    |
| B                                                                                                                                                                                                            | 1.78             | —14.5 | 4.12             | —16.0 |  |  | 30 |
| C                                                                                                                                                                                                            | 1.72             | —30.7 | 4.32             | —21.0 |  |  |    |
| G                                                                                                                                                                                                            | 1.74             | —27.3 | 4.29             | —20.0 |  |  |    |
| H                                                                                                                                                                                                            | 1.93             | —19.1 | 3.85             | —16.0 |  |  |    |

TABLE 6

| Processing of photosensitive material M with image receiving materials A2 and A3. Processing temperature: 32° C.; CO <sub>2</sub> -exposure: 0h; Number of materials that have been processed before: 0. |                  |       |                  |       |  |  |    |
|----------------------------------------------------------------------------------------------------------------------------------------------------------------------------------------------------------|------------------|-------|------------------|-------|--|--|----|
| Processing solution                                                                                                                                                                                      | Mat. A2          |       | Mat. A3          |       |  |  |    |
|                                                                                                                                                                                                          | D <sub>max</sub> | Gamma | D <sub>max</sub> | Gamma |  |  |    |
| B                                                                                                                                                                                                        | 1.73             | —36.0 | 4.47             | —19.0 |  |  | 40 |
| C                                                                                                                                                                                                        | 1.72             | —34.0 | 4.48             | —20.0 |  |  |    |
| G                                                                                                                                                                                                        | 1.71             | —36.0 | 4.50             | —17.0 |  |  |    |
| H                                                                                                                                                                                                        | 1.88             | —25.0 | 4.20             | —23.0 |  |  |    |

From tables 1-6 it can be seen that the fresh processing solutions according to the present invention are better than the comparative solutions particularly at low temperature. Especially good results are obtained with processing liquids H and F that contain DEAPD as the only alkanol amine.

TABLE 7

| Processing of photosensitive material N with image receiving materials A2 and A3. Processing temperature: 23° C.; CO <sub>2</sub> -exposure: 48h; Number of materials that have been processed before: 0. |                  |       |                  |       |  |  |    |
|-----------------------------------------------------------------------------------------------------------------------------------------------------------------------------------------------------------|------------------|-------|------------------|-------|--|--|----|
| Processing solution                                                                                                                                                                                       | Mat. A2          |       | Mat. A3          |       |  |  |    |
|                                                                                                                                                                                                           | D <sub>max</sub> | Gamma | D <sub>max</sub> | Gamma |  |  |    |
| A                                                                                                                                                                                                         | 1.82             | 17.2  | 3.19             | 20.6  |  |  | 60 |
| B                                                                                                                                                                                                         | 1.81             | 15.0  | 3.08             | 17.0  |  |  |    |
| C                                                                                                                                                                                                         | 1.64             | 9.9   | 2.47             | 14.0  |  |  |    |
| F                                                                                                                                                                                                         | 1.75             | 25.4  | 3.69             | 17.2  |  |  |    |

TABLE 7-continued

| Processing of photosensitive material N with image receiving materials A2 and A3. Processing temperature: 23° C.; CO <sub>2</sub> -exposure: 48h; Number of materials that have been processed before: 0. |                  |       |                  |       |  |  |   |
|-----------------------------------------------------------------------------------------------------------------------------------------------------------------------------------------------------------|------------------|-------|------------------|-------|--|--|---|
| Processing solution                                                                                                                                                                                       | Mat. A2          |       | Mat. A3          |       |  |  |   |
|                                                                                                                                                                                                           | D <sub>max</sub> | Gamma | D <sub>max</sub> | Gamma |  |  |   |
| G                                                                                                                                                                                                         | 1.83             | 15.0  | 2.91             | 16.0  |  |  | 5 |
| H                                                                                                                                                                                                         | 1.90             | 24.0  | 3.52             | 21.0  |  |  |   |

TABLE 8

| Processing of photosensitive material M with image receiving material A2. Processing temperature: 23° C.; CO <sub>2</sub> -exposure: 30h; Number of materials that have been processed before: 0. |                  |       |  |  |  |  |    |
|---------------------------------------------------------------------------------------------------------------------------------------------------------------------------------------------------|------------------|-------|--|--|--|--|----|
| Processing solution                                                                                                                                                                               | Mat. A2          |       |  |  |  |  |    |
|                                                                                                                                                                                                   | D <sub>max</sub> | Gamma |  |  |  |  |    |
| B                                                                                                                                                                                                 | 1.89             | —15.2 |  |  |  |  | 20 |
| C                                                                                                                                                                                                 | 1.64             | —6.9  |  |  |  |  |    |
| G                                                                                                                                                                                                 | 1.89             | —11.6 |  |  |  |  |    |
| H                                                                                                                                                                                                 | 1.99             | —18.6 |  |  |  |  |    |

Tables 7 and 8 show that the processing liquids according to the present invention are less susceptible to CO<sub>2</sub>-absorption particularly processing solutions containing DEAPD as the only alkanol amine.

TABLE 9

| Processing of photosensitive material N with image receiving materials A1, A2 and A3. Processing temperature: 23° C.; CO <sub>2</sub> -exposure: 0h; Number of materials that have been processed before: 100. |                  |       |                  |       |                  |       |    |
|----------------------------------------------------------------------------------------------------------------------------------------------------------------------------------------------------------------|------------------|-------|------------------|-------|------------------|-------|----|
| Processing solution                                                                                                                                                                                            | Mat. A1          |       | Mat. A2          |       | Mat. A3          |       |    |
|                                                                                                                                                                                                                | D <sub>max</sub> | Gamma | D <sub>max</sub> | Gamma | D <sub>max</sub> | Gamma |    |
| A                                                                                                                                                                                                              | 1.63             | 14.8  | 1.75             | 14.1  | 3.21             | 13.2  | 35 |
| B                                                                                                                                                                                                              | —                | —     | 1.66             | 18.4  | 3.40             | 20.3  |    |
| C                                                                                                                                                                                                              | —                | —     | 1.75             | 16.0  | 3.33             | 16.2  |    |
| D                                                                                                                                                                                                              | 1.76             | 10.4  | 1.84             | 12.2  | 2.92             | 13.6  |    |
| E                                                                                                                                                                                                              | 1.75             | 13.6  | 1.85             | 15.4  | 3.25             | 16.0  |    |
| F                                                                                                                                                                                                              | —                | —     | 1.72             | 21.0  | 4.02             | 18.3  |    |
| G                                                                                                                                                                                                              | —                | —     | 1.70             | 19.7  | 3.29             | 20.2  |    |
| H                                                                                                                                                                                                              | —                | —     | 1.65             | 27.6  | 3.86             | 27.5  |    |

TABLE 10

| Processing of photosensitive material M with image receiving materials A2 and A3. Processing temperature: 23° C.; CO <sub>2</sub> -exposure: 0h; Number of materials that have been processed before: 100. |                  |       |                  |       |  |  |    |
|------------------------------------------------------------------------------------------------------------------------------------------------------------------------------------------------------------|------------------|-------|------------------|-------|--|--|----|
| Processing solution                                                                                                                                                                                        | Mat. A2          |       | Mat. A3          |       |  |  |    |
|                                                                                                                                                                                                            | D <sub>max</sub> | Gamma | D <sub>max</sub> | Gamma |  |  |    |
| B                                                                                                                                                                                                          | 1.72             | —12.9 | 2.64             | —20.1 |  |  | 50 |
| C                                                                                                                                                                                                          | 1.73             | —11.6 | 2.70             | —21.9 |  |  |    |
| G                                                                                                                                                                                                          | 1.75             | —13.3 | 2.83             | —21.9 |  |  |    |
| H                                                                                                                                                                                                          | 1.86             | —16.6 | 3.01             | —25.7 |  |  |    |

Tables 9 and 10 show that the processing liquids according to the present invention show a slower exhaustion than the comparative solutions.

I claim:

1. An aqueous alkaline processing liquid suitable for use in the silver complex diffusion transfer reversal process wherein complex silver ions are transferred to an image receiving element which comprises a silver halide solvent and is substantially free from developing agents characterized in that said liquid comprises 3-(N,N-diethylamino)propane-1,2-diol in an amount between 0.1 mol/l and 1.5 mol/l and wherein said liquid is free of phosphate ions.

2. An aqueous alkaline processing liquid according to claim 1 further comprising at least one second alkanolamine.

3. An aqueous alkaline processing liquid according to claim 2 wherein said second alkanol amine is N-methyl-ethanolamine.

4. A method for obtaining an image comprising information-wise exposing a photographic material containing a silver halide emulsion layer and (a) developing agent(s) and developing said information-wise exposed photographic material according to the silver complex diffusion transfer reversal process while in contact with an image receiving layer containing physical development nuclei wherein complex silver ions are transferred to an image receiving element using an aqueous alkaline processing liquid substantially free of developing agents and phosphate ions and comprising a silver halide solvent and 3-(N,N-diethylamino)propane-1,2-diol in a total amount between 0.1 mol/l to 1.5 mol/l.

5. A method according to claim 4 wherein said aqueous alkaline processing liquid further comprises at least one second alkanolamine.

6. A method according to claim 5 wherein said second alkanolamine is N-methyl-ethanolamine.

7. A method for obtaining an image comprising information-wise exposing a photographic material containing a silver halide emulsion layer and developing said information-wise exposed photographic material according to the silver complex diffusion transfer reversal process while in contact with an image receiving layer containing physical development nuclei wherein complex silver ions are transferred to an image receiving element using an aqueous alkaline processing liquid comprising a silver halide solvent, 3-(N,N-diethylamino)propane-1,2-diol, at least one developing agent of the p-hydroxybenzene type and phosphate ions from 0.0 mol/l to 0.03 mol/l.

8. A method according to claim 7 wherein said 3-(N,N-diethylamino)propane-1,2-diol is present in an amount of 0.05 mol/l to 1.5 mol/l.

9. A method according to claim 7 wherein said aqueous alkaline processing liquid further comprises at least one second alkanolamine.

10. A method according to claim 9 wherein said second alkanolamine is N-methyl-ethanolamine.

\* \* \* \* \*